

1

3,212,895  
**STABILITY OF RAPID-PROCESSED  
PHOTOGRAPHIC MATERIALS**

Jean Barbier, Paris, and Jean-Pierre Fauchille, Vincennes, France, assignors to Eastman Kodak Company, Rochester, N.Y., a corporation of New Jersey  
No Drawing. Filed Dec. 20, 1960, Ser. No. 77,009  
5 Claims. (Cl. 96—61)

This invention relates to photography and more particularly to an improvement in stabilization of rapidly processed photographic materials.

Rapid processing of photographic materials is known. Stabilization of such rapidly developed silver images is known using solutions of compounds such as alkali metal and ammonium thiocyanates and thiosulfates, or alkali metal and ammonium compounds of thiourea and thioglycolic acid. In rapid processing it is customary to eliminate the fixing and washing steps and to stabilize the developed image by treatment with a solution of a compound which does not react with metallic silver and which forms a light-stable silver complex by reaction with undeveloped silver halide. While the methods known in the art are satisfactory for the stabilization of silver images which are not to be stored under adverse conditions, there is the disadvantage that such silver images tend to fade when stored under conditions of high temperature and humidity. Consequently, rapid processing has had little appeal for use in preparing prints that are to be stored for any length of time, for example, in office files.

It is, therefore, an object of the present invention to provide rapid-processing emulsions capable of being stabilized to produce prints having improved stability to high temperature and humidity. A further object is to provide a rapid-processing method for silver halide emulsion layers which produces prints having improved stability to storage at high temperature and humidity.

These objects are accomplished by the method described herein which includes treating a rapidly processed silver halide emulsion layer with a solution of an alkali or ammonium bisulfite and formaldehyde. The select mixture of our invention can advantageously be incorporated in the silver halide emulsion directly or it can be used as a separate treating bath after conventional stabilization with a stabilizing compound such as ammonium thiocyanate. In either event, the select mixture is effective in preventing fading on storage of rapidly processed prints in a humid environment. Particularly subject to fading has been thiocyanate-stabilized silver images which have been known to become almost illegible after a few months storage in a humid environment. We have now found that rapid processed prints can be preserved using the novel combination of our invention such that copies can be obtained which have a stability nearly equal to a photograph treated by standard sodium thiosulfate and wash means. The improved print stability obtained using particular combinations of this invention was not obtained where either of the components of the combination was employed alone.

The stabilizing process customarily used in the preparation of rapidly processed prints which are further stabilized according to our invention is described in Brice U.S. Patent 2,448,857, issued September 7, 1948, and in Broughton et al. U.S. Patent 2,614,927, issued October 21, 1952. According to the process, a silver halide photographic emulsion, preferably a gelatin-silver halide emulsion, is exposed in the usual way and developed with a suitable silver halide developing solution. After develop-

2

ment, the excess developing solution present on the surface of the print is removed by any convenient means such as squeegee, and the print is then treated with a stabilizing solution. The purpose of the stabilizing agent is to make the undeveloped silver halide substantially incapable of change on further light exposure. The stabilizing agent must be a compound which does not react with metallic silver and which forms a light-stable, silver complex by reaction with the undeveloped silver halide in the emulsion layer. Stabilizing agents described for this purpose in Yackel application Serial No. 594,589 and in Broughton et al. U.S. Patent 2,614,927, issued October 21, 1952, are compounds containing double-bonded sulfur or an SH linkage, such as alkali metal and ammonium thiosulfates and thiocyanates, thiourea and thioglycolic acid. Additional stabilizing agents which may be employed in the stabilizing of layers preserved according to our invention are described in Russell U.S. Patent 2,453,346, issued November 9, 1948. In the use of such stabilizing agents the resulting silver complex should be light colored or transparent so that there is no interference with the viewing or printing of the final image.

According to our invention any of the above-described stabilizing agents can be employed. However, alkali metal and ammonium thiocyanate stabilizing agents are preferred. In the practice of our invention we may use a thiocyanate stabilizing compound, such as ammonium thiocyanate, and in addition, we further stabilize so as to give an increased preservation of the silver image using a combination of a bisulfite and formaldehyde. The bisulfite compounds of our invention can be alkali metal or ammonium bisulfites, e.g., sodium metabisulfite, potassium metabisulfite, ammonium metabisulfite, or ammonium, potassium, or sodium bisulfite. The formaldehyde is conveniently used as an aqueous solution. The concentration of the water-soluble alkali bisulfite compounds can vary as an ingredient in the aqueous solution of the formaldehyde-bisulfite mixture from as little as 1.0 percent to as high as 15 percent of the total weight of the aqueous solution. The percentage of formaldehyde in the formalin-bisulfite solution can vary from as little as 1.5 percent to as high as about 8 percent of the total volume. When the select mixture is added to the emulsion, suitable proportions of a solution containing from about 5 to about 10 percent of bisulfite and 4 to 6 percent formaldehyde can be used. This solution when added to the emulsion is added in an amount from about 8 percent to about 12 percent of the total emulsion volume. Alternatively, the bisulfite, e.g., sodium bisulfite or potassium metabisulfite can be added in solution directly to the emulsion separately from the formaldehyde solution if the latter is added to the emulsion in excess of the amount needed for emulsion-hardening purposes. Preferably, however, the bisulfite is first dissolved in the aqueous formaldehyde solution prior to addition to the emulsion, e.g., where thiocyanate-stabilized images are to be treated by bathing in the bisulfite-formaldehyde mixture, the bisulfite is present in an amount of from about 5 percent to about 10 percent of the weight of a 4 percent formaldehyde aqueous solution. These concentrations are based on a treatment or immersion time in the bath of about 30 seconds. Lower concentrations can be used with longer application or immersion times. The time will vary with the nature of the film, that is, the grain size, chemical composition, and with the temperature of treatment. Formalin which is an aqueous solution containing about 37 percent formaldehyde by weight is a convenient source of the formaldehyde.

The process of our invention is particularly adaptable to improving the keeping characteristics of developed silver images which have been stabilized with solutions of thiocyanate although the treatment also improves the image stability where other stabilizing compounds, such as sodium thiosulfate have been used. It was found that the smaller the grain size of the emulsions, the more critical and difficult it became to insure satisfactory stability. It is deduced from this fact that the image deterioration is a surface phenomenon.

The emulsions used in this invention can advantageously be hardened emulsions. The emulsions may be hardened with any suitable hardener for gelatin such as formaldehyde, a halogen-substituted aliphatic acid such as mucobromic acid as described in White U.S. Patent 2,080,019, or by compounds such as those described in U.S. Patents 2,725,294, 2,725,295, and 2,725,305. The emulsions may be coated on paper or other opaque supports or on any of the well known transparent supports such as cellulose nitrate, cellulose acetate, polyethylene terephthalate, polystyrene, polycarbonates, etc.

The developing agents which are incorporated into the emulsions, rapidly-processed and stabilized according to our invention, can be developing agents such as 3,4-dihydroxydiphenyl, 2,3-dihydroxydiphenyl, and hydroquinone compounds (e.g., hydroquinone, chlorohydroquinone, methylhydroquinone, etc.), 3-pyrazolidone (e.g., 1-phenyl-3-pyrazolidone, 4-methyl-1-phenyl-3-pyrazolidone, 4,4-dimethyl-1-phenyl-3-pyrazolidone, etc.). These developing agents can be incorporated into the emulsion substantially as indicated in the examples herein described.

My invention will be further illustrated by reference to the following specific examples:

#### Example 1

The following example illustrates a manner of improving the stability of rapidly-processed photographic prints according to our invention.

An emulsion suitable for use in our invention was made as follows:

Solutions were made of (a) 25 grams of gelatin in 1 liter of water at 40° C., (b) 100 grams of silver nitrate in 500 cc. of water at 20° C., and (c) 35 grams of sodium chloride in 500 cc. of water. Solutions (b) and (c) were simultaneously run into solution (a) at a uniform rate while stirring the latter over a period of about 10 minutes. Solution (b) was not allowed to run in faster than (c). Thereafter, 150 grams of gelatin in 1200 cc. of water at 40° C. were added. 25 grams of 3,4-dihydroxydiphenyl were then dissolved in 250 cc. of methyl alcohol. This solution was slowly added to the above mixture. The emulsion was hardened by using a suitable gelatin hardening agent such as formaldehyde. Following the hardening of the emulsion, 300 grams of a 4 percent formaldehyde solution containing 5 percent by weight of sodium metabisulfite was added with stirring. The emulsion was then coated on a paper support over an area of about 500 square feet. Samples of the dried product were then exposed in a number of ways to a subject, including by contact with or projection of a negative and by reflex exposure with a subject comprising printed matter on a paper base. Thereafter the exposed samples of the element containing a developing agent in the emulsion were treated for about 60 seconds in an aqueous alkaline solution of the following composition:

|                                  | Grams |
|----------------------------------|-------|
| Sodium carbonate monohydrate     | 50    |
| Sodium hydroxide                 | 5     |
| Sodium thiosulfate (crystalline) | 2     |
| Potassium bromide                | 12    |
| Water to make 1 liter.           |       |

The above alkaline developing solution was applied with a sponge. After development, the surface was

squeeged and the unfixed element was then treated for about 60 seconds with the following solution of a stabilizing agent applied with a sponge:

|                           |       |     |
|---------------------------|-------|-----|
| Ammonium thiocyanate      | grams | 320 |
| Sodium fluoride           | grams | 4   |
| Chrome alum (2% solution) | ml    | 100 |
| Acetic acid (99.5%)       | ml    | 40  |
| Sodium metabisulfite      | grams | 50  |
| Water to make 1 liter.    |       |     |

- 10 The developing and stabilizing treatments can also be accomplished by other means, e.g., by rolling the exposed element down onto a pad moistened with the processing solution. After processing, the samples made and processed as outlined in this example were compared to control strips that were identically made and processed, except that no addition of metabisulfite and formaldehyde was made to the emulsion. The strips were hung in a wet oven at 120° F. and 98 percent relative humidity. The silver images on the test strips containing the sodium metabisulfite and formalin were still clearly legible after nine days, whereas in the control strips the image faded in about seven hours.

#### Example 2

25 The following example illustrates the improvement in silver image stability obtained by treatment of thiocyanate-stabilized rapidly-processed images in a treating solution containing sodium metabisulfite and formalin.

30 An emulsion suitable for use in our invention was made as follows:

35 Solutions were made of (a) 25 grams of gelatin in 1 liter of water at 40° C., (b) 100 grams silver nitrate in 500 cc. of water at 20° C., and (c) 35 grams of sodium chloride in 500 cc. of water. Solutions (b) and (c) were simultaneously run into solution (a) at a uniform rate while stirring the latter over a period of about 10 minutes; solution (b) preferably not being allowed to run in faster than (c). Thereafter, 150 grams of gelatin in 1500 cc. of water at 40° C. were added. To this solution, then, was added 250 cc. of methyl alcohol containing 25 grams of 3,4-dihydroxydiphenyl. The emulsion was then hardened with formaldehyde and coated on paper support over an area of about 500 square feet. The product was then exposed, developed, and stabilized as described in Example 1.

40 After stabilization, various strips of the material were treated using a variety of reducing agents including hydroquinone, ascorbic acid, formalin, and a solution of sodium metabisulfite and formaldehyde. The following table shows the various results obtained where these compounds were used in a treating solution following stabilization in ammonium thiocyanate. The treated paper strips and untreated controls were stored at 120° F. and a relative humidity of 98 percent. Treatment of the paper strips was accomplished by rolling the stabilized element down onto a pad which was moistened with the preserving compound in solution. The following test results were obtained:

| 60                                           | Treatment after stabilization control | Stability at 120° F.,<br>98% RH |
|----------------------------------------------|---------------------------------------|---------------------------------|
| No after treatment                           |                                       | Image lasted 2 hours.           |
| 5% Hydroquinone solution                     |                                       | Image lasted 4 hours.           |
| 5% Sodium metabisulfite solution             |                                       | Image lasted 7 hours.           |
| 5% Ascorbic acid solution                    |                                       | Image lasted 5 days.            |
| 4% Formaldehyde solution                     |                                       | Image lasted 3 days.            |
| 4% Formaldehyde and 5% sodium metabisulfite. |                                       | Image lasted more than 8 days.  |

70 These results show the improved image stability obtained when an ammonium thiocyanate stabilized rapidly-processed silver image is treated with the combination of this invention comprising sodium metabisulfite and formaldehyde.

75 The advantages of our process are apparent from the examples in that an improved durability of certain rapid-

ly-processed silver images is obtained where the additive of our invention is employed.

It is apparent that some reaction occurs between the bisulfite and formaldehyde when aqueous solutions thereof are mixed to produce an alkali metal (or ammonium) formaldehyde bisulfite (sometimes called a sulfoxylate), and that this product can be added to the emulsion, or treating bath, instead of the mixtures mentioned above. It is important that a source of bisulfite ion and formaldehyde be available in the stabilization treatment, and the source thereof is not important. Of course, when a metabisulfite is dissolved in water, this provides the bisulfite ion ( $\text{HSO}_3^-$ ). A metabisulfite is essentially an anhydride of a bisulfite, e.g.,  $\text{Na}_2\text{S}_2\text{O}_5$  is the anhydride of  $\text{NaHSO}_3$ .

As mentioned, our emulsions are preferably gelatin-silver halide emulsions. However, we are not limited thereto since other water-permeable organic colloid vehicles may be used for dispersing the silver salt and developing agent, e.g., polyvinyl alcohol, partially hydrolyzed polyvinyl esters and cellulose esters, etc.

It is apparent from the foregoing description of our invention that a substantial proportion of the silver compounds remains in the emulsion after the stabilizing treatment. This differs from the customary fixing and washing in which the intent is to remove the residual silver halide from the emulsion.

The invention has been described in detail with particular reference to preferred embodiments thereof, but it will be understood that variations and modifications can be effected within the scope and spirit of the invention as described hereinabove and as defined in the appended claims.

We claim:

1. In a rapid process for the formation of a silver image in a silver halide photographic layer which comprises:

- (a) exposing said layer,
- (b) developing a silver image in said layer with a silver halide developing agent, and
- (c) stabilizing said silver image and silver halide by treating said layer with a solution of a compound selected from the class consisting of the alkali metal thiocyanates, the alkali metal thiosulfates, ammonium thiocyanate, ammonium thiosulfate, thiourea and thioglycolic acid, until substantially all the residual silver halide is converted to a light stable silver complex, the improvement comprising the step of

(1) contacting the stabilized silver image and silver complex in said layer with an aqueous solution of formaldehyde and a compound selected from the class consisting of an alkali metal bisulfite, ammonium bisulfite, an alkali metal metabisulfite and ammonium metabisulfite to preserve the said stabilized image and silver complex in said layer against fading produced by storage at elevated temperatures and elevated humidity.

2. The process of claim 1 in which the preserving step comprises the contacting of a rapidly developed and stabilized photographic silver halide element with an aqueous solution of formaldehyde and sodium bisulfite.

5 3. A light-sensitive photographic element for rapid processing comprising a support having coated thereon a silver halide emulsion containing:

- (a) a silver halide developing agent, and
- (b) a silver image preservative comprising aqueous formaldehyde and a member selected from the class consisting of an alkali metal bisulfite, an alkali metabisulfite, ammonium bisulfite and ammonium metabisulfite.

10 4. A light-sensitive photographic element for rapid processing comprising a support having coated thereon a silver halide emulsion containing:

- (a) a silver halide developing agent selected from the class consisting of 3,4-dihydroxydiphenyl, 2,3-dihydroxydiphenyl, a hydroquinone and a 3-pyrazolidone, and
- (b) a silver image preservative comprising aqueous formaldehyde and sodium formaldehyde bisulfite addition complex.

15 5. A light-sensitive photographic element for rapid processing comprising a support having coated thereon a silver halide emulsion containing:

- (a) a silver halide developing agent selected from the class consisting of 3,4-dihydroxydiphenyl, 2,3-dihydroxydiphenyl, a hydroquinone and a 3-pyrazolidone, and
- (b) a silver image preservative comprising aqueous formaldehyde and ammonium formaldehyde bisulfite addition complex.

#### References Cited by the Examiner

##### UNITED STATES PATENTS

|              |       |                  |       |         |
|--------------|-------|------------------|-------|---------|
| 710,568      | 10/02 | Eichengrun       | ----- | 96-61   |
| 1,941,852    | 1/34  | Brunken          | ----- | 96-111  |
| 40 1,954,512 | 4/34  | Allison          | ----- | 96-61   |
| 2,571,725    | 10/51 | Kimball et al.   | ----- | 96-85   |
| 2,614,927    | 10/52 | Broughton et al. | ----- | 96-61   |
| 2,845,349    | 7/58  | Schwarz          | ----- | 96-66   |
| 45 2,865,745 | 12/58 | Chan et al.      | ----- | 96-28   |
| 2,902,367    | 9/59  | Welliver et al.  | ----- | 96-66   |
| 3,030,209    | 4/62  | Henn et al.      | ----- | 96-66 X |
| 3,079,858    | 3/63  | Haydn et al.     | ----- | 96-35   |
| 3,080,230    | 3/63  | Haydn et al.     | ----- | 96-95   |

##### OTHER REFERENCES

Noller, Chemistry of Organic Compounds, pp. 199-200, Saunders and Co., Philadelphia (1951).  
Yule, Journal of the Franklin Institute, vol. 239, pp. 221-230, 1945.

55 NORMAN G. TORCHIN, Primary Examiner.

HAROLD N. BURSTEIN, ABRAHAM H. WINKELSTEIN, Examiners.